

## UNITED STATES PATENT OFFICE.

HENRY N. CASE, OF OAK PARK, ILLINOIS, ASSIGNOR TO SEARS, ROEBUCK AND CO., OF CHICAGO, ILLINOIS, A CORPORATION OF NEW YORK.

## COATED PAPER AND SUBSTANCE FOR COATING THE SAME.

No Drawing.

Application filed March 5, 1919. Serial No. 280,751.

To all whom it may concern:

Be it known that I, HENRY N. CASE, a citizen of the United States, residing at Oak Park, in the county of Cook and State 5 of Illinois, have invented an Improved Coated Paper and Substance for Coating the Same, of which the following is a specification.

This invention relates to a paper base 10 coated on both sides with material capable of being etched to produce reliefs suitable for use as matrices in subjecting printing plates to the McKee process. One of the greatest difficulties in making such coated 15 paper is to avoid conditions which will prevent the finished matrix from being the exact size of the printing plate with which the matrix is to be used. Another serious difficulty is to make the coatings of uniform thickness.

The object of this invention is to produce a high-grade coated paper, and to provide a bath for coating the paper which eliminates the difficulties heretofore encountered 25 in manufacturing such paper.

The process for applying the coating material to the paper is claimed in my co-pending applications, Serial Nos. 280,750 and 370,542 filed March 5, 1919 and April 1, 30 1920, respectively, and no claim to such process is therefore made herein.

While the paper base may be of any suitable character, I have obtained good results with a paper stock having a base weight of 35 24 lbs. per ream of 17x22 sheets; a thickness of four one-thousandths of an inch, with very slight calendering; all-rag fiber, preferably all cotton; capable of standing a 7 degree Baumé bleach for five minutes without becoming too tender to stand rough handling; which will not shrink or expand one one-hundredth of an inch per foot in either direction when soaked in water and dried in the air; and which is beater-sized 40 and tub-sized, the sizing being free from grease. The paper may be of any suitable width, as, for example, 18 inches, and is preferably supplied in the form of rolls of convenient diameter.

Without intending to limit myself to any

particular ingredients or to any particular proportions thereof, it may be stated that good results have been obtained with a solution or mixture formed of the following ingredients:

55

Clay, 39 lbs.; water for the clay, 28 lbs.; gelatine, 74 oz.; water for the gelatine, 15 pints.

The clay should be clean, dry and not coarse; a good grade of English china clay 60 is satisfactory.

The water and the gelatine should be free from oil and grease. Since practically all commercial gelatines contain a small percentage of fatty acid, a small quantity of 65 alkali, as, for example, 90 c. c. of a 10% solution of sodium hydroxide, should be used in making up a batch of coating material.

It is necessary that the overlay shall 70 exactly register with the printing plate for which it is made, from which it follows that the overlay in drying after the etching operation should return with great precision to its original dimensions. I have discovered that the jelly strength of the size 75 is a factor in the shrinkage of the etching. When size that is low in jelly strength is used, the overlay when being dried after the etching operation will shrink below its 80 original dimensions. Glue and gelatin give the best results.

If the coating solution is made up one day to be used the following day a preservative should be added. A small quantity 85 of phenol may be used for this purpose.

It is desirable that there be a distinction between the color of the coating and the color of the paper base, in order that the operator may know when the paper has 90 remained in the etching solution for the necessary length of time. For this purpose a small quantity of some suitable coloring matter may be employed with the other ingredients, as, for example, 120 grams of 95 10% paranitraniline red. This color is fast to the chloride of lime etching solution. No color should be used which is water-resistant.

In order to make the coating smooth and 100

uniform, it is desirable to mix and grind the ingredients in a suitable mill, as, for example, a paint mill, the hopper of which is large enough to hold an entire batch.

- 5 The hopper and the receiving receptacle should be heated to keep the material from jellifying during the grinding.

In making up the coating, a layer of clay is placed in the bottom of the hopper of the

- 10 mill; some of the water for the clay is then added, then a second layer of clay, and so on. Before all of the clay and water are added, the coloring material is mixed into a little of the water and added to the clay.

- 15 The clay may be allowed to soak for two hours or longer.

The gelatine is thoroughly moistened with the specified quantity of water and allowed to soak for, say, two hours. The alkali and

- 20 preservative are then added to the gelatine, and the gelatine dissolved by applying heat.

The clay after soaking is stirred thoroughly; the gelatine is then poured into the hopper of the mill through an 80-mesh sieve,

- 25 after which the batch is again stirred. The mill is then started.

When the grinding is completed, the application of heat to the container for the batch is discontinued and the batch permitted to jellify over night.

- 30 The following morning heat is again applied to the batch so as to cause the latter to melt. After straining the batch and skimming off the bubbles, the viscosity of the batch is measured and water added until, after thorough

35 stirring, the batch is of the desired viscosity. The alkali causes an increase in the viscosity of the batch, which action increases with the time of standing. For this reason, an excess

- 40 of alkali must not be used.

Any suitable apparatus may be used to apply the coating material to the paper, as, for example, the construction illustrated in my copending application Serial No. 280,

- 45 750, filed March 5, 1919.

In order to prevent the formation of small pits in the applied coating, it is necessary to keep the coating material free from particles of lint, greasy particles, or particles

- 50 not necessarily greasy but not easily wet by water. The grinder, the coating machine, and all utensils must be kept free from oil,

grease and other substances not readily miscible with water.

- 55 In handling a coating as high in sizing as the one herein described, it is difficult to prevent foaming. The difficulty may, however, be obviated or cured by avoiding violent agitation, by repeated skimming, and

60 by using two compartments in the coating machine so that the compartments in which the paper is coated receives its supply from the bottom of the compartment into which the coating is poured.

- 65 To prevent variations in the thickness of

the coating, which manifest themselves in horizontal streaks, it is necessary that the paper be drawn through the bath at a uniform rate. If the paper be drawn through the bath too rapidly, streaks will form in all 70 directions.

The paper may be dried in any suitable way, after which it is cut into sheets of convenient size, as, for example, 12x18 or

- 17 $\frac{1}{2}$ x22 $\frac{1}{2}$ . The sheets are then calendered in

75 any suitable manner, as, for example, by means of the plating method, a number of sheets being placed between zinc plates, and the whole run back and forth between two large cylinders under great pressure. In

- 80 drying, the overlay paper should shrink to a point slightly but definitely below the initial size of the paper base. To obtain a coating which satisfactorily fulfills this requirement,

85 the proportion of the gelatinous sizing to the clay body, and also the jelly strength of the sizing, should be such that the shrinkage of the whole coating composition should be slightly but definitely greater

- 90 than the expansion of the paper base which occurred when the latter became wet during the coating process. If the coating did not shrink when drying, the paper base would

not be allowed to shrink to the proper extent, and consequently shrinkage would occur in drying after etching. By properly

- 95 proportioning the sizing and the clay body, and using sizing of proper jelly strength, the coated paper is caused to shrink slightly below the original dimensions of the paper

100 base. This excess shrinkage is corrected when the paper is slightly stretched by the plating process. It is obvious that any

- 105 slight variation in the grain size or other properties of the clay or in the jelly strength

110 of the sizing would necessitate a repropor-

- 115 tioning of the ingredients to secure the de-

sired result. Thus a coated paper is ob-

- 120 tained which will not stretch or shrink on being a second time wetted and dried, as after the etching process.

The coating material and the process herein disclosed produce a paper coated on both sides with a smooth, etchable coating of uniform thickness, and which will not shrink

- 115 after etching.

While I have herein referred to the paper as adapted for use in making McKee matrices, it will be understood that the paper has

- various other uses.

120 I claim as my invention:

1. A coating composition for use in manufacturing coated paper consisting of clay, gelatine, alkali and water (in approximately the following proportions: clay, 39 125 pounds, water for the clay, 28 pounds, gela-

- 125 tine, 74 ounces, water for the gelatine, 15 pints, and 90 c. c. of a 10% solution of sodium hydroxide), and a coloring material.

2. A coating composition for use in manu-

- 130

facturing coated paper consisting of clay, gelatine and water in approximately the following proportions: clay, 39 pounds, water for the clay, 28 pounds, gelatine, 74 5 ounces, water for the gelatine, 15 pints.

3. A coating composition for use in manufacturing coated paper comprising English china clay and grease-free gelatine.

4. A coating composition for use in manufacturing coated paper comprising a mineral and gelatine free from grease and oil.

5. A bath for coating overlay paper comprising water, powdered clay, a gelatinous sizing, an alkali to eliminate all traces of 15 grease, and a preservative for the sizing.

6. A paper base coated with a composition capable of being etched and comprising

powdered clay incorporated in a grease free gelatinous sizing containing a preservative.

7. An etchable coating composition for 20 paper comprising grease free sizing material of high jelly strength, and inert body material incorporated with said sizing material, the mixture of sizing and body material being in such proportions as to produce a factor 25 of shrinkage of the coat in drying after the coating operation, slightly but definitely greater than the expansion of the paper base when it becomes wet during the coating operation.

In testimony whereof, I have hereunto set 30 my hand.

HENRY N. CASE.